

## UNITED STATES PATENT OFFICE

1,930,110

## PROCESS FOR THE PRODUCTION OF FLUORESCENT OR PHOSPHORESCENT SUBSTANCES

Emil Rupp, Glienicke, Germany, assignor to  
General Electric Company, a corporation of  
New YorkNo Drawing. Application February 1, 1932,  
Serial No. 590,321, and in Germany February  
5, 1931

## 4 Claims. (Cl. 204—1)

The present invention relates to processes for the production of fluorescent or phosphorescent substances.

It is now known that such substances consist of a principal material such as zinc sulphide, zinc sulphate, calcium sulphide or common salt with an addition of a heavy metal such as copper, manganese, or bismuth. Hitherto the metal constituent has been added to the principal material in the order of 0.1 to 1%, parts by weight, by the method of fusing or sintering, using a suitable flux material in this latter method.

The object of the present invention is to produce a fluorescent or phosphorescent material consisting of the commonly known principal materials and heavy metals by an electrical transference of the metal constituent to the principal material. Still further objects and advantages, attaching to the device and to its use and operation will be apparent to those skilled in the art from the following particular description.

In accordance with this object the invention consists in the new and novel features of operation and the new and original arrangements and combinations of steps in the process hereinafter described and more particularly set forth in the claims.

The principal material, such as one of those disclosed above, is arranged between the electrodes, said electrodes consist of that same metallic material which is to be incorporated in the principal material. The principal material, having poor electrical conducting characteristics, is brought to a high temperature when an appreciable current is applied to said electrodes which increases its electrical conductivity. Metallic particles from the electrodes are carried by the electric discharge between said electrodes and are deposited in the principal material interposed between said electrodes. This transposition of the metallic particles from the electrodes to the principal material interposed therebetween may be conveniently described as a kind of electrolytic effect and will be referred to hereinafter as electrolysis. Either direct or alternating current can be used as desired. In order that the fluorescent or phosphorescent material produced have maximum activity the quantity of deposited metallic material must reach a certain optimum for certain materials, this depends on the nature of the particular principal material and the particular metallic material used. The yield in this process, as in all electrolysis, is

proportional to the product of the current strength and the time.

The following examples are given by way of illustrating practical applications of the present invention:

*Example 1.*—The materials used are sodium chloride (NaCl) and manganese. A crystal of rock salt is placed between two manganese electrodes. The apparatus is then heated in a furnace to a temperature of 450° C. to increase the electrical conductivity of said sodium chloride while a current of sufficient voltage to cause 5–10 milli-amperes to flow through the rock salt crystal is applied to said electrodes. This is continued for approximately 30 minutes. The crystal is then cooled and upon being irradiated glows with an intense yellow color.

*Example 2.*—The materials used are zinc sulphide and copper. Commercial zinc sulphide powder is pressed between copper electrodes and electrolyzed at 600° C for about half an hour by a current of 10 to 20 milli-amperes. When cooled and irradiated the powder sends out a green glow.

A plurality of different metallic materials may be introduced into a single body of principal material by this process by substituting for one set of electrodes of a certain metallic material another set of electrodes of a different metallic material during the carrying out of the process, and further, particularly where alternating current is used, electrodes of different metallic material may be used for the same purpose.

Although I have shown and described and have pointed out in the annexed claims certain novel features of the invention, it will be understood that various omissions, substitutions and changes in the several steps of the process and its operation may be made by those skilled in the art without departing from the broad spirit and scope of the invention.

What I claim as new and desire to secure by Letters Patent of the United States is:—

1. A process for the production of phosphorescent material consisting of a principal material and a metallic addition which comprises the steps of interposing a body of the principal material, which is a poor electrical conductor, between two electrodes consisting of that metal desired to be incorporated in said principal material, heating said electrodes and said body of principal material to increase the electrical conductivity of said principal material and applying a suitable electric current to said electrodes for a sufficient period to transfer a desired

66

65

70

75

80

85

90

95

100

105

110

quantity of the metallic material from said electrodes to said principal material.

2. A process for the production of phosphorescent material consisting of sodium chloride and an addition of manganese which comprises the steps of interposing a body of sodium chloride, which is a poor electrical conductor, between two electrodes consisting of that metal desired to be incorporated in said principal material, heating said electrodes and said body to a temperature of approximately 450° C. to increase the electrical conductivity of said body of sodium chloride and applying an electrical current of approximately 5-10 milli-amperes to said electrodes for approximately 30 minutes to effect a transposition of manganese particles from said electrodes to the body of sodium chloride interposed between said electrodes.

20

3. A process for the production of phosphorescent material consisting of zinc sulphide and an addition of copper which comprises the steps of interposing a body of zinc sulphide, which is a poor electrical conductor, between two copper electrodes, heating said electrodes and said body to a temperature of approximately 600° C. to increase the electrical conductivity of said body of zinc sulphide and applying an electrical current of approximately 10-20 milli-amperes to said electrodes for approximately 30 minutes to effect a transposition of copper particles from said electrodes to the body of zinc sulphide interposed between said electrodes.

80

4. A phosphorescent, fluorescent body comprising sodium chloride having incorporated therein an electrically deposited addition of manganese.

EMIL RUPP.

85

90

95

25

100

30

105

35

110

40

115

45

120

50

125

55

130

60

135

140

145

150